

## UNITED STATES PATENT OFFICE

LEON W. EBERLIN, OF ROCHESTER, NEW YORK, ASSIGNOR TO EASTMAN KODAK COMPANY, OF ROCHESTER, NEW YORK, A CORPORATION OF NEW YORK

## ULTRA-VIOLET SENSITIVE PAPER

No Drawing.

Application filed April 27, 1931. Serial No. 533,365.

This invention relates to photo-sensitive paper, the sensitivity of which lies chiefly in the ultra-violet.

It is desirable for certain actinometric purposes to have a light sensitive material which reacts to the near ultra-violet rays without being appreciably affected by the rest of the spectrum. Specifically, such a material may be used to demonstrate or dose the ultra-violet radiation of sunlight and of various artificial light sources, particularly those used therapeutically. It is an object of this invention to produce such a paper.

Under the influence of ultra-violet light, ortho-nitrobenzaldehyde undergoes molecular rearrangement to ortho-nitroso-benzoic acid. By using a suitable indicator with ortho-nitrobenzaldehyde, I have been able to produce a paper which is sensitive primarily to the ultra-violet and which has very little sensitivity in the visible spectrum. On exposure to ultra-violet light this paper gives within a short time a visible color change showing the transformation or rearrangement just described.

A test paper suitable for determining the intensity of ultra-violet light may be made by dipping sheets of unsized paper into a solution of

Example I

Ortho-nitro-benzaldehyde----- 1 gram  
Lacmoid ----- 0.1 gram  
Ethyl alcohol----- 100 c. c.

Under the influence of ultra-violet this paper changes from blue to pink, and an exposure of about one minute is normally sufficient to produce a good color change.

Another suitable formula is the following:

Example II

Ortho-nitro-benzaldehyde----- 1 gram  
Brom-thymol blue----- 0.1 gram  
Gelatin ----- 0.1 gram  
Acetone----- 100 c. c.

Papers may be made with such solutions by either dipping or floating the sheets of paper upon the solution, then withdrawing and drying. Sized paper will, as a rule, not

be satisfactory for this purpose, the sizing materials in them interfering with the indicator. Unsized papers and those containing no fillers of any kind will be preferable. A suitable material is filter paper.

I have found that the sensitivity of a paper made in the manner just described has a sensitivity lying almost entirely in the range of about 2480 to 3650 Ångstrom units, and is very little affected by visible light.

It will be understood that I do not limit myself by the particular examples given, especially so far as indicators are concerned, as it will be evident that other substances are available for producing a satisfactory result.

What I claim as my invention and desire to secure by Letters Patent of the United States is:

1. A photo-sensitive sheet sensitive primarily to the ultra-violet comprising ortho-nitrobenzaldehyde.

2. A photo-sensitive sheet sensitive primarily to the ultra-violet comprising ortho-nitrobenzaldehyde and an indicator.

3. A photo-sensitive sheet sensitive primarily to the ultra-violet comprising ortho-nitrobenzaldehyde and an indicator, which gives on exposure a visible color change.

Signed at Rochester, New York, this 20th day of April, 1931.

LEON W. EBERLIN.

80  
85  
90  
95  
100

80  
85  
90  
95  
100